

Dec. 16, 1941.

P. E. BLANCHFIELD ET AL

2,266,390

BALL

Filed Nov. 12, 1940



INVENTORS  
Paul E. Blanchfield  
Raphael A. Stafford

BY *Feyrer and Mack*  
ATTORNEYS

## UNITED STATES PATENT OFFICE

2,266,390

## BALL

Paul E. Blanchfield and Raphael A. Stafford,  
Chicopee, Mass., assignors to A. G. Spalding &  
Bros. Inc., Chicopee, Mass., a corporation of  
Delaware

Application November 12, 1940, Serial No. 365,228

15 Claims. (CL 273—60)

This invention relates: to play balls, particularly to baseballs; to resilient materials useful in the manufacture of baseballs and other objects of controlled resiliency; to processes for impregnating yarns with macromolecular organic chemicals; and to processes and structure for controlling the length of flight of a baseball.

Reference is made to the "sluggish baseball" invention of which we are among the inventors; said invention is described in an application filed by John B. Dickson, Raphael A. Stafford and Paul E. Blanchfield, Serial No. 350,378, filed August 3, 1940. The present invention generally discloses another type of sluggish baseball or the like and a method of making the same.

Present-day baseballs have evolved over a considerable period of time and those used by baseball leagues, such as National, American and International, are closely standardized for size and weight by definite and well-established rules. Moreover, great care has been exercised to provide a ball having suitable resistance to deformation, to provide sufficient softness in the ball to prevent injury to the hands in catching the ball, and to provide other desirable qualities.

One standard baseball which has come into extensive use consists primarily of a leather cover superposed upon a center, including divers yarn windings about a main core consisting of an outer core concentrically enclosing a cork sphere or inner core  $\frac{5}{8}$  of an inch in diameter, the hollow spherical outer core being approximately  $1\frac{1}{8}$  inches in diameter and/or  $4\frac{1}{8}$  inches in circumference.

This invention relates particularly to the yarn windings for play balls. In such products there is ordinarily provided: an inner wool yarn winding sometimes known as a chunk; an intermediate wool winding; an outer wool yarn winding; the above-mentioned inner, intermediate and outer windings constituting the resilient winding; and a protective winding of cotton string of considerably smaller thickness interposed between the so-called outer winding and a cover.

Because of the development of the skill of baseball players in recent years there have been an objectionably large number of heavy hitters having the ability to hit a baseball so far as to assure a home run, or at least far enough to decrease the likelihood of catching a "fly." The batting averages have been increased by this decreased likelihood of a long hit being caught. The spectator's interest in baseball has lessened because of the increased number of home runs and the higher batting averages which have been attained.

To prevent an objectionably large number of home runs, some attempts have been made recently to provide a satisfactory "short," "dead" or "sluggish" ball. These attempts have included 5 the provision of: looser or softer windings of yarn; thicker cords in the seams between the cover parts to absorb some of the blow from the bat; and bulkier cords in the seams between the cover parts to increase the wind resistance and to thereby cut down the flight.

While softer or looser windings of yarn did result in more sluggish baseballs, such balls were impractical because they were adversely deformed very easily. Thicker or bulkier cords for the 15 seams did not decrease the flight of balls sufficiently to produce the desired result of making the game more interesting to the spectators by reducing the number of home runs and decreasing the batting averages of the players.

20 Heretofore there have been divers proposals for impregnating windings such as the protective winding with very resilient materials such as rubber latex, but such proposals have never been of commercial importance and such proposals have 25 provided balls having a considerably increased flight attributable perhaps to the latex impregnation.

Further, it has been thought impracticable to 30 impregnate the resilient winding because it has been thought that the impregnation would prevent the ball from complying with the narrow weight limitations relating to baseballs. With the present invention no major or adverse weight increase is built into the ball.

35 In the past it has been thought that only wool yarn was satisfactory for the resilient winding of a baseball. Numerous attempts have been made to substitute cheaper materials and some effort has been made to provide a material having better properties. However, no substitute for wool 40 has been developed, and it is still the material which is ordinarily used in the resilient winding of a baseball. With the present invention it has been found possible to use other than all-wool 45 yarns.

In making the tests to determine the reactance to hitting of the different balls, a hitting machine driven by falling weights was used. This machine propelled a standard or "league" baseball 50 after making allowances for such variables as wind velocity, about 350 feet, which is long enough to produce a home run in many ball parks. A large number of balls have been tested against the standard distance of 350 feet. Until the 55 development of the present invention and the

aforementioned invention in application Serial No. 350,378, so far as applicants are aware, there have been no "short" balls or those flying less than the standard distance for a standard blow except certain balls having undesirable properties of lack of balance, tendency to be easily deformed and other objectionable qualities.

As used in this specification, the speed with which the resilient winding restores itself to normal shape after being deformed by an impact, such as developed by a bat hitting a baseball is called "restoration speed."

As used in this specification "resiliency" of a material refers to its tendency to move in counteraction to a force. For small forces such as dropping an object from a height of 100 inches, or hitting it with a projectile moving at the rate of 23 feet per second, the term "rebound" is used. For large forces such as dropping an object 625 feet or hitting it with a projectile moving at the rate of 200 feet per second the term "reactance" is used, as are the terms "long" and "short." "Durability" refers to the quality of resisting deformation or misshapeliness under continued whacking or frequent impact, and not to oxidation resistance or the like. Heretofore it has been thought that low resiliency of rubbery materials was necessarily accompanied by a small degree of durability.

It is an important object of the present invention to provide a process for manufacturing a baseball having a shorter flight than a conventional league baseball.

Another important object is to provide a baseball conventional in substantially all respects excepting that said baseball possesses a shorter flight than ordinary league balls.

Still another object of the present invention is to provide resilient fibrous masses having less resiliency than ordinary fibrous masses.

It is a further object to provide a process by means of which a completed yarn winding of a semimanufactured baseball can be simply and inexpensively impregnated with a macromolecular organic material.

It is a further object of the present invention to provide a "sluggish" baseball having an unusually great resistance to misshapeliness and having the property of withstanding use for a longer period of time than conventional baseballs.

Other objects of the present invention are:

To provide a method of controlling the sluggishness of a baseball so that as the ability of baseball players improves and other conditions require it baseballs of suitably sluggish properties or having a suitably shorter flight can be manufactured.

To provide a means of controlling the resiliency of fibrous masses in such a manner as to assure a slower rate of restoration than fibrous masses ordinarily have.

To provide a baseball making use of a small quantity of costly yarn.

To make possible the use of yarn other than all-wool yarn in the resilient winding of a baseball.

A most important feature of the present invention is the provision of a process of impregnating components of resilient windings of baseballs with macromolecular organic materials for the purpose of reducing the reactance of the resilient windings, thereby reducing the flight of the baseballs.

Other features of the present invention include:

The provision of fibrous masses impregnated with macromolecular organic materials having a small amount of resiliency.

The provision of durable resilient materials having low reactance and rebound as materials for the inner and outer cores with specially impregnated resilient windings.

The use of large diameter cores in a baseball with specially impregnated resilient windings.

The use of numerous other features apparent from a consideration of the specification.

In the drawing:

Figure 1 is a plan view of a complete baseball.

Fig. 2 is a sectional view taken along line 2-2 of Fig. 1.

Fig. 3 is an enlarged view of a section of Fig. 2.

Fig. 4 is a diagrammatic representation of apparatus in which yarn and/or a completed yarn winding may be impregnated.

Before describing the present improvements and mode of operation thereof in detail it should be understood that the invention is not limited to the details of construction and arrangement of parts shown in the accompanying drawing, or to the details of the formulae herein described, which are merely illustrative of the present preferred embodiments, and the phraseology employed is for the purpose of description and not of limitation.

Referring now in detail to the drawing, which shows the present preferred embodiments of the invention embodied in a baseball, it will be seen that an inner core 10 is positioned within an outer core 11, the two members combining to constitute a core 12. A chunk 13 or inner winding is wound about the core 12. Superposed about the chunk 13 is an intermediate winding 14 about which is an outer winding 15. The windings 13, 14 and 15 constitute a resilient winding 16 discussed in detail hereinafter. About the resilient winding 16 is superposed a protective winding 17 usually of cotton string.

The core 12, resilient winding 16 and protective winding 17 constitute a ball center 18. A leather cover 19 is superposed upon the ball center 18 to form a completed baseball 20.

Of particular importance, the present invention includes the provision of an especially impregnated fibrous material, such as yarn, said especially impregnated material serving to retard the flight of a ball. The chunk 13, for example, may contain a partial impregnation 13a. In Fig. 4 is shown apparatus for impregnating yarn with a deadening material, for example, with organic macromolecular materials such as hereinafter described. A strand of yarn 21 may be passed into a deadening solution 22 beneath a rod 23, and out of the solution 22, which is contained in a vat 24. It is desirable that the impregnated yarn 25 be quickly and thoroughly dried. For this purpose a conventional drying oven 26 may be provided. The impregnated yarn 25 passes through the drying oven 26. After the impregnated yarn 25 has been dried it may be reeled up upon a spool 27 for future use. The deadening material preferably has the characteristic of retarding the reactance springiness of the yarn, without making the same rigid or "stony." Accordingly, such materials as Celluloid are outside the scope of the present invention.

Instead of impregnating the strand of yarn separately it is preferable to partially impregnate 75 a semimanufactured baseball. As shown in Fig.

4, a semimanufactured baseball 28 comprising the core 12 and at least one or more of the windings 13, 14 and/or 15 may be submerged in the deadening solution 22 and may be placed upon a support 29. The impregnated semimanufactured baseball 30 may be quickly and thoroughly dried in any suitable and conventional manner, as for example, by placing it in the drying oven 26.

The deadening solution 22 for impregnating the fibrous material, such as certain of the individual strands of yarns, or preferably the windings of yarn upon the semimanufactured balls, comprises a suitable deadening material and a suitable solvent. Below are listed some of the formulae provided for this purpose by the present invention:

| Percentage deadening agent by weight | Percentage solvent by weight |
|--------------------------------------|------------------------------|
| Per cent                             | Per cent                     |
| Cellulose acetate 8.5                | Acetone 91.5                 |
| Tenite II 8.5                        | Acetone 91.5                 |
| Lucite 8.5                           | Ethylene dichloride 91.5     |
| Thiokote 8.5                         | Ethylene dichloride 91.5     |
| Vistanex 8.5                         | Petroleum naphtha 91.5       |

It has been found that when a portion of the resilient winding 16 is impregnated with a deadening agent, such as, for example, an organic macromolecular material, the flight of the baseball 20 made with such a winding is substantially less than that of an ordinary league baseball. For example, it has been found that when the chunk 13 of an ordinary semimanufactured and regular league baseball is partially impregnated with cellulose acetate, as by dipping a chunk 13 (formed about a core 12) into the above cellulose acetate solution, then dried and completed in the usual manner, the flight of the baseball is reduced approximately 5 feet. It should be particularly noted that the sluggish baseball is like a regular league baseball in every respect as to the size and composition of each component, excepting for the impregnation of the chunk, which impregnation produces 5 feet of reduction in flight. An impregnation of Tenite II, a special kind of cellulose butyrate, reduces the flight of a corresponding baseball 6 feet. It has also been found that when Lucite, a methylmethacrylate resin, is used as the impregnating and deadening material the flight of the corresponding baseball is reduced 7 feet. When Thiokote is used as impregnating and deadening material the flight of the corresponding baseball is reduced approximately 3 feet. Especially good results were obtained when the deadening solution contained Vistanex, an isobutylene polymer, as the impregnating compound. When the chunk 13 was partially impregnated with Vistanex, the flight of the baseball 20 was reduced 10 feet.

The comparative reductions in flight mentioned in the preceding paragraph were obtained by using a baseball 20 identical with a league baseball, excepting for the impregnation 13a of the chunk 13. However, it has been found that when the impregnation is effected at a point closer to the cover 19 of the ball 20 a greater reduction in flight is accomplished. For example, it was found that when the intermediate winding 14 was impregnated with Vistanex the reduction in flight was approximately 12 feet, and that when the outer winding 15 was impregnated with Vistanex the reduction in flight was from 12 to 15 feet.

It should be particularly noted that, according to the present invention, at least some cotton, rayon or part-wool yarns may be used instead of using only all-wool yarns as is customary in the manufacture of a baseball. When the yarn or semi-manufactured baseball is impregnated with organic macromolecular material such as Vistanex, Lucite or Tenite, it is not necessary to use all-wool yarn. Because of the high price of wool and the relatively low price of cotton, rayon and other nonwool materials this feature makes it possible to produce an impregnated ball even more inexpensively than a ball having an all-wool resilient winding.

According to the present invention it is not necessary to penetrate the entire thickness of a winding in impregnating it, and it is only necessary to obtain a penetration constituting approximately one-half of the thickness of the winding to satisfactorily or appreciably reduce the flight of the corresponding baseball as compared with a nonimpregnated baseball. Such an impregnation can easily be produced by dipping for approximately one minute in a deadening solution such as described hereinabove. When the intermediate winding 14 is dipped, the chunk 13 will also be partially impregnated unless the dipping is accurately controlled.

Similarly, it has been found that when at least a portion of the resilient winding 16 is made of impregnated yarn 25, complete penetration of the deadening material is not necessary and that a partially impregnated yarn is very satisfactory for use in accordance with the principles of this invention. Ordinarily the greatest economies can be effected in the manufacturing process by impregnating the semimanufactured ball 28 instead of impregnating the yarn 21 because when separately impregnated yarn 25 is used, it is sometimes necessary to adjust the winding machines and to alter the number of turns for each of the windings, to change the tension of winding, and to modify other factors influencing the winding. Whenever the resilient winding 16 includes separately impregnated yarn 25 or at least one impregnated winding 13, 14 or 15 (yarn impregnated after winding on the ball), the final resilient winding 16 is referred to as a sluggish winding.

Now, of particular importance, it has been found that the effect of providing a sluggish core 12 and the effect of providing a sluggish winding 16 is at least cumulative and under certain conditions, more than cumulative. Accordingly, it is possible to provide a sluggish core 12 such as described in a copending application (of John B. Dickson, Raphael A. Stafford and Paul E. Blanchfield) Serial No. 350,378, filed August 3, 1940, with a sluggish winding, as described hereinbefore, and to thereby have a ball of greatly retarded flight, and to shorten the flight of the ball a much greater extent than is possible with either the sluggish core or the sluggish winding alone.

The present invention contemplates including the provision of specially impregnated fibrous material, such as yarn, upon any of the sluggish cores set forth in detail in said application Serial No. 350,378.

The copending application describes the use of inner cores of: cork, for most of the experiments; compressed gas, which was found to provide a more sluggish baseball than cork inner cores; kapok, which was found to be superior

to cork for a sluggish inner core; Vistanex, which was found to be especially effective as a sluggish inner core; conventional diameter of  $\frac{3}{8}$  of an inch; and larger diameter, as for example cores  $1\frac{1}{8}$  inches in diameter, and  $1\frac{1}{2}$  inches in diameter for the compressed gas inner core.

The copending application describes the use of: outer cores of rubber having a larger diameter than normal, resulting in a longer flight of the ball; outer cores of rubber smaller than conventional, resulting in a longer flight of the ball; outer cores of low resilient material resulting in shorter flights of the ball; outer cores of low resilient material of enlarged diameter, resulting in a considerably reduced flight, it being established that increasing the diameter of the core up to two inches resulted in further reductions in the flight of the baseball; outer cores of low rebound materials such as described hereinafter.

The copending application describes low rebound compositions such as those indicated by the following formulae:

|                           |    |    |    |    |    |    |    |    |
|---------------------------|----|----|----|----|----|----|----|----|
| Polyisobutylene           | 18 | 51 | 41 | 29 | —  | —  | —  | —  |
| Polyxylene                | —  | —  | —  | —  | 53 | 48 | 46 | 39 |
| Polyalkene-sulfide        | 45 | —  | —  | 16 | —  | —  | —  | —  |
| Rubber                    | 4  | 11 | 13 | 28 | 22 | 20 | 31 | 26 |
| Fillers and curing agents | 33 | 28 | 46 | 27 | 25 | 32 | 23 | 35 |

The copending application also describes the use of a Koroseal outer core, Koroseal being a polyvinylchloride material containing a large quantity of plasticizer.

Said copending application describes sluggish baseballs having a shortness in flight of from 2 to 35 feet. According to the present invention, the control of the sluggishness is effected not merely by the core size and composition, but also by the impregnation of the resilient winding. By this method it is possible to produce a baseball considerably shorter in flight than those balls described in detail in said copending application. For example, if a ball 35 feet short were provided with an impregnated outer winding, it would be approximately 50 feet short, or approximately 15% short.

It has been found that the impregnated yarn, either in the form of a strand of yarn, or in the form of a semi-manufactured baseball, may be dried in the air or in an oven. The drying rate affects the nature of gelation of the deadening agent. The drying rate sometimes influences the flight of the baseball and the durability thereof is somewhat affected thereby. Best results are obtained by rapidly drying the impregnated yarn in a drying oven. Moreover, the oven method speeds up the manufacturing process.

In one form the process for making ball components includes the steps of making a core; treating a yarn with a deadening material; and winding yarn on the core. This process may also be augmented with the step of forming a cover on the component.

In another form the process provided by the present invention includes the steps of forming a sluggish core; forming one or more windings on the core; applying deadening material to one or more of said windings; and forming a cover on the windings.

A further and at present preferred process includes steps of making a core; forming one or more windings of yarn on the core; impregnating one or more of said windings with a deadening

ing material; and forming a cover on said winding.

Although not preferred, any of the plurality of windings 13, 14 and/or 15 may be replaced by a single winding, or may be replaced by a shell of compressed fibrous material such as kapok, and may be impregnated with deadening materials in the manner hereinbefore set forth in connection with the divers windings.

10 Obviously the fibrous material could be coated by precipitation from a suspension, or adhesion from molten mass, or other methods instead of adsorption from a solution.

15 Although it is not certain, it is believed that the explanation of the reduction in flight attributable to the sluggish winding is due to the fact that the restoration speed of the sluggish winding is less than the restoration speed of an unimpregnated winding. The restoration speed of a 20 latex impregnated winding, being greater than the unimpregnated winding, excludes such materials from the scope of the present invention. Other highly resilient materials such as polybutadiene, polychloroprene, gelatinized glue chromate, etc., are also meant to be excluded. Substantially all other organic macromolecular materials, sometimes hereinafter designated as non-resilient organic macromolecular materials, are believed to be effective impregnated agents, although of course certain ones would not be used 25 because of their cost, odor, instability, low solubility, etc. Other materials than macromolecular organic materials, such as tar or waterglass, would also function as deadening agents, according 30 to the present invention.

Other variations and modifications may be made within the scope of this invention and portions of the improvements may be used without others.

40 Having thus described the invention what is claimed as new is:

1. A play ball including a resilient member of fibrous material, said fibrous material containing in at least certain portions a deposit of deadening material adapted to reduce the reactance of said resilient member.

2. In a play ball the combination of a core; a fibrous member superposed about said core; a deposit of deadening material in at least certain portions of said fibrous member, said deadening material being adapted to impart a reduced reactance to said fibrous member; and a cover on said ball.

3. In a play ball the combination of a sluggish core; a fibrous member superposed about said core; a deposit of deadening material in at least certain portions of said fibrous member, said deadening material being adapted to impart a reduced reactance to said fibrous member; and a cover on said ball.

60 a cover on said bar.

4. A resilient member in a resilient article  
adapted to possess a slow restoration speed, low  
resiliency, cushioning properties and great dura-  
bility, said member consisting of fibrous material  
65 at least partially impregnated with a deadening  
material chosen from the class consisting of poly-  
isobutylene, polyalkenesulfide, polyvinylchloride,  
polymethylmethacrylate and cellulose acetate.

5. A play ball including a member of reduced reactance, said member consisting of fibrous material at least partially impregnated with organic macromolecular material adapted to impart to said member a reduced reactance.

6. A play ball including a core; a cover; and  
75 interposed between the core and cover a member

of reduced reactance, said member consisting of fibrous material at least partially impregnated with deadening material chosen from the class consisting of polyisobutylene, polymethylmethacrylate, cellulose acetate, polyalkenesulfide and polyvinylchloride.

7. In a play ball the combination of a core; a cover; and interposed between the core and cover at least one yarn winding with at least one of said yarn windings being at least partially impregnated with deadening material adapted to impart to said yarn winding a reduced reactance.

8. A play ball including a member of reduced reactance, said member consisting at least partially of cellulosic material at least partially impregnated with polyisobutylene.

9. A play ball comprising a member of reduced reactance, said member consisting at least partially of cellulosic material at least partially impregnated with deadening material.

10. A sluggish baseball including a sluggish inner core; a sluggish outer core; at least one winding on said outer core; a deadening material deposit in at least some portion of at least one of said windings; and a cover.

11. In a play ball the combination of a cover, a fibrous member at least partially impregnated with a deadening agent; and an outer core consisting of rubber, suitable fillers and curing agents, and a modifying agent of rubber soluble synthetic organic macromolecular material of relatively small resiliency with respect to rubber.

12. In a play ball the combination of an inner core having a diameter greater than  $\frac{7}{8}$  of an inch, said inner core consisting of a material of small resiliency; an outer core having a diameter greater than  $1\frac{1}{8}$  inches, said outer core consisting of a composition of small resiliency; a fibrous member superposed about said outer core, said fibrous member being at least partially impregnated with a deadening agent.

13. A play ball including an outer core consisting of suitable curing agents, fillers, rubber and at least 25% modifying agent chosen from the class consisting of polyisobutylene, polyalkenesulfide, polyxylene and polyvinylchloride; a fibrous member superposed about said outer core; a deposit of deadening agent in at least some portions of said fibrous member, said deadening agent being chosen from the class consisting of polyisobutylene, polymethylmethacrylate, polyalkenesulfide, polyvinylchloride and cellulose acetate; and a cover.

14. In a play ball the combination of a cover; a core; yarn windings between the cover and the core; and a deposit of deadening material on at least certain sections of said yarn windings.

15. In a play ball the combination of a cover; a core; a fibrous member between the cover and the core; and a deposit of deadening material on at least certain sections of said fibrous member.

PAUL E. BLANCHFIELD.  
RAPHAEL A. STAFFORD.